

# United States Patent Office

3,103,472  
Patented Sept. 10, 1963

1

3,103,472

ELECTROLYTIC PRODUCTION OF ALUMINUM  
Harvey L. Slatin, New York, N.Y., assignor to Timax  
Associates, New York, N.Y., a partnership  
No Drawing. Filed Dec. 23, 1959, Ser. No. 861,431  
6 Claims. (Cl. 204—67)

This invention relates to the production of aluminum by fusion electrolysis.

This application is a continuation-in-part of my application concerned with the Electrolytic Production of Aluminum, Serial No. 613,718, filed October 3, 1956, now U.S. Patent No. 2,919,234, dated December 29, 1959.

The instant invention provides a process for the production of aluminum by fusion electrolysis using an aluminum halide, such as aluminum chloride as a source of feed material.

The art contains records of attempts to produce aluminum from  $AlCl_3$  by electrolysis using an electrolyte composed of  $AlCl_3$  dissolved in alkali and/or alkaline earth halides.  $AlCl_3$  is a volatile solid subliming at about 178° C. Although its vapor pressure may be suppressed in molten alkali chloride eutectic baths at or about the melting point of aluminum (659.7° C.),  $AlCl_3$  is readily distilled from such baths. As a consequence these processes are operated at low temperatures or under a positive pressure. In the former instance, aluminum is deposited as a solid commingled with electrolyte that is difficult to separate from the metal crystals. In the latter process, the equipment and labor are expensive and not proved practical.

Great interest in the use of  $AlCl_3$  as a raw material is stimulated by the fact that present processes based on electrolysis of alumina consume from 0.6 to 1.0 pound of carbon per pound of aluminum. In addition, the high temperatures of operation cause severe corrosion, shorten equipment life and add to the cost of production.  $AlCl_3$  obviates these shortcomings.

This invention overcomes the disadvantages of presently used electrolytes containing  $AlCl_3$  by providing a process wherein little, if any,  $AlCl_3$  is found in the electrolyte. The process comprises electrolyzing a fused salt bath composed of alkali halides between a dependent carbon or graphite anode and a cathode of molten aluminum which is denser than the electrolyte bath, simultaneously with the electrolysis feeding into the liquid cathode gaseous  $AlCl_3$ . Under such circumstances, chlorine is discharged at the insoluble inert anode and aluminum is deposited and accumulated at the cathode.

The rate of  $AlCl_3$  feed is synchronized with the rate of deposition of aluminum so that virtually all of the  $AlCl_3$  fed to the cathode is completely consumed. Although three faradays of electricity are theoretically required to decompose the  $AlCl_3$  into its elements, in actual practice somewhat more than three faradays are required. The current efficiency will be above 95% reaching as high as 98.5%.

The following example will illustrate the invention:

A eutectic mixture of  $NaCl$ — $KCl$  melting at about 650° C. to which about 10% by weight of  $CaF_2$  was added was fused in a covered graphite lined crucible. Due to the small size of the laboratory equipment used, auxiliary external heating was provided. A high fired alumina collecting dish was placed at the bottom of the graphite liner. Aluminum metal was added piece by piece to the bath until a pool of about 1" in thickness had formed in the dish. A hollow graphite tube was lowered into the bath until it extended below the surface of the aluminum which was made cathode. The graphite liner was made anode. The cell was purged by air and vented to a chlorine absorber. With the commencement of electrolysis, gaseous  $AlCl_3$  was fed into the cell below the Al level

2

via the hollow graphite tube and cathode lead. The current flow through the cell was maintained at about 200 amperes. The rate of feed was erratic, but substantially no  $AlCl_3$  was found in the anode chlorine gas. At the end of 90 minutes of feeding and electrolyzing, the feed was stopped and the current discontinued. The weight of total feed was about 350 grams. A metal button was separated from the frozen salts and analyzed. The results are as follows:

10 Temperature of electrolysis \_\_\_\_\_ 700–750° C.  
Purity of  $AlCl_3$  \_\_\_\_\_ <97%.  
Cathode current density \_\_\_\_\_ 16–32 amps./in.<sup>2</sup>.  
Anode current density \_\_\_\_\_ 2.7 amps./in.<sup>2</sup>.  
Purity of aluminum \_\_\_\_\_ 99.26% Al.

The electrolyte is composed of cations more electro-positive than aluminum with respect to the halogens. Although the alkaline earth metal halides are useful, sodium and potassium halides are preferred. Similarly, although halides in general may be used, the chlorides are preferred. Small additions of alkali and/or alkaline earth fluorides seem to improve the electrolyte. The alkali chlorides are not consumed in the process but losses due to entrainment and volatilization require replenishment from time to time. The preferred anode is graphite, but carbon or other insoluble conductors may be used.

The raw material feed may be any of the halides of aluminum and as a practical matter the chloride is preferred as it is the easiest and cheapest to produce from common available ores and the easiest to handle.

30 Aluminum chloride is fed to the cathode preferably as a gas or vapor. All lines leading from the boiler or sublimer to the cell must be lagged to prevent condensation and plugging of the lines. It may be desirable to pass an inert gas through the lines with the  $AlCl_3$  gas to keep the lines open, or to stir the melts, or afford a means for controlling the feed rate in small cells. The feed rate should be controlled so that all the  $AlCl_3$  is consumed and so that substantially no  $AlCl_3$  breaks through the surface of the aluminum cathode or distills into the chlorine phase. In the event that the rate of feed is greatly in excess of the rate of aluminum deposition, some aluminum chloride may find its way into the electrolyte. No irreparable harm is done, but it is advisable to control the feed rate to prevent  $AlCl_3$  contaminating the chlorine gas stream or clogging the vents. The feed lines are lined internally with graphite, but it has been found that carbides, such as silicon carbides, are superior. The  $AlCl_3$  should be kept free of water or moisture since it hydrolyzes readily leaving insoluble and highly corrosive residues.

50 The temperature of electrolysis should be 50–100° C. above the melting point of aluminum in order to permit tapping of the aluminum product. The lower temperature of operation promotes current efficiency, lengthens cell life and reduces corrosion rates.

55 The current density at the liquid cathode may be varied over a wide range from a fraction of an ampere per square inch to over 25 amperes per square inch. Similarly, the anode current density may be varied from a fraction of an ampere per square inch to over 10 amperes per square inch. However, for the smoothest operation and for maximum efficiency, the anode current density should be maintained below 7 amperes per square inch and the cathode current density below 10 amperes per square inch, 6–7 amperes per square inch are preferred.

60 The reaction of the instant invention is not known precisely and the applicant does not wish to be committed to any theory. The  $AlCl_3$  is not fed to the electrolyte at all. The fact that little if any finds its way into the electrolyte points to its decomposition before reaching the salt bath. It may be that sodium (in an alkali chloride electrolyte) is deposited momentarily at the interface of

the electrolyte and the liquid cathode. The sodium at once reacts with the  $\text{AlCl}_3$  or the product of the reaction of aluminum with the  $\text{AlCl}_3$ . The reactions may be represented by:



However, from back E.M.F. readings, it would appear that no free sodium is deposited and that the aluminum is deposited by primary electrolysis. In any event, unless the  $\text{AlCl}_3$  is bubbled into the liquid aluminum coincidentally with the passage of electrolyzing current, the process becomes impractical if not inoperative.

I claim:

1. A process for the production of aluminum by fusion electrolysis comprising electrolyzing a fused salt bath comprising at least one of the group consisting of the alkali and alkaline earth halides, said bath having a lesser density than molten aluminum, said electrolysis being effected between an insoluble anode and a liquid aluminum cathode submerged in said electrolyte, simultaneously feeding gaseous aluminum halide below the surface of said cathode, at a rate to confine the aluminum halide essentially to the liquid cathode, reducing the aluminum ion to aluminum solely in said cathode to maintain the fused salt bath free of aluminum halide and passing the halide ion to said bath, thereby discharging a corresponding volatile halide gas at said insoluble anode and accumulating aluminum at the bottom of said electrolytic cell.

2. A process for the production of aluminum by fusion electrolysis comprising electrolyzing a fused salt bath composed of at least one of the group consisting of the alkali and alkaline earth chlorides and fluorides, said bath hav-

ing a lesser density than molten aluminum, said electrolysis being effected between an insoluble anode and a liquid aluminum cathode submerged in said electrolyte, simultaneously feeding gaseous aluminum chloride below the surface of said cathode at a rate to confine the aluminum chloride essentially to the liquid cathode reducing the aluminum ion to aluminum solely in said cathode to maintain the bath free of aluminum chloride and passing the chloride ion to said bath, thereby discharging chlorine at said insoluble anode and accumulating aluminum at the bottom of said electrolytic cell.

5. A process for the production of aluminum as set forth in claim 2, wherein the rate of feed of said aluminum chloride is synchronized with the number of faradays passing through said cell.

10 6. A process for the production of aluminum as set forth in claim 2, wherein said electrolyte comprises the alkali metal chlorides of sodium and potassium.

20 7. A process for the production of aluminum as set forth in claim 2, wherein said electrolysis is conducted using an anode current density below about 7 amperes per square inch and a cathode current density of about 6 amperes per square inch.

25 8. A process for the production of aluminum as set forth in claim 2, wherein a fluoride of the group consisting of the alkali and alkaline earth fluorides is added to the electrolyte.

References Cited in the file of this patent

UNITED STATES PATENTS

1,297,946 Weaver ----- Mar. 18, 1919

FOREIGN PATENTS

687,758 Great Britain ----- Feb. 18, 1953

745,530 Great Britain ----- Feb. 29, 1956